

## UNITED STATES PATENT OFFICE.

JAMES S. MARRS AND ROBERT M. MORRIS, OF ST. LOUIS, MISSOURI.

## LEATHER-SURFACE-REPAIR COMPOSITION.

No Drawing.

Application filed March 28, 1921. Serial No. 456,186.

*To all whom it may concern:*

Be it known that we, JAMES S. MARRS and ROBERT M. MORRIS, citizens of the United States, residing in the city of St. Louis and State of Missouri, have invented a new and useful Leather-Surface-Repair Composition, of which the following is a specification.

The object of our invention is the production of a leather surface repair composition to be applied to scratches, cuts, imperfections and damaged or injured surfaces of the leather uppers of shoes or boots in a heated state, and which when so applied and subjected to pressure and rubbing action of a heated spatula, becomes firmly incorporated in the injured surface of the leather for repairing the defect.

The composition consists of a mixture of carnauba wax, refined beeswax, shellac wax, ceresine wax, dry shellac, turpentine and a color base made up of either pigment, chrome and earthy colors such as dry colors or pigments, lamp black or carbon black.

In preparing the composition, we prefer to use the ingredients in approximately the following proportions, namely:

One ounce of carnauba-wax, one ounce refined beeswax, one ounce shellac-wax, one ounce Venice liquid turpentine, one ounce dry shellac and a color base sufficient to suitably color the composition. Good results may be obtained, however, when Burgundy pitch, gum thus, or terebinthina are substituted for the liquid turpentine.

The ceresine wax is used without the carnauba wax when a cheaper product is desired.

The above ingredients are thoroughly mixed together in a heated state in a suitable vessel to the proper consistency. The color base is added after the other ingredients have been thoroughly agitated or mixed to give blended color to the repair composition. After all the ingredients have been thoroughly mixed and the composition

brought to the proper consistency, it is poured into containers and allowed to set, after which it is ready for use by being applied to a scratched, cut, or otherwise injured leather surface by means of a heated spatula, or knife blade and subjected to pressure and a rubbing action for working it into a homogeneous state.

Our composition is very efficient, is impervious to water, adheres without blooming to an injured leather surface when applied thereto, takes polish freely, and, as a whole, when applied by the heat process, possesses in a very high degree all the desired properties of a leather repair composition.

What we claim is:

1. A leather surface repair composition, comprising substantially one ounce carnauba wax, one ounce beeswax, one ounce shellac wax, one ounce dry shellac, one ounce turpentine and a color base.

2. A leather surface repair composition, comprising substantially one ounce carnauba wax, one ounce beeswax, one ounce shellac wax, one ounce dry shellac, one ounce ceresine wax, one ounce turpentine and a color base.

3. A leather surface repair composition, comprising one ounce of carnauba wax, one ounce refined beeswax, one ounce Venice turpentine, one ounce shellac and a color base.

4. A leather surface repair composition, comprising one ounce of carnauba wax, one ounce refined beeswax, one ounce Venice turpentine, one ounce shellac, one ounce ceresine wax and a color base.

5. A leather surface repair composition, comprising substantially one ounce beeswax, one ounce shellac wax, one ounce dry shellac, one ounce ceresine wax, one ounce turpentine and a color base.

In testimony whereof, we have hereunto signed the specification.

JAMES S. MARRS.  
ROBERT M. MORRIS.